

## UNITED STATES PATENT OFFICE

2,407,489

## ELECTRODEPOSITION OF ZINC

Allen G. Gray, Rocky River, Ohio, assignor to E. I.  
du Pont de Nemours & Company, Wilmington,  
Del., a corporation of Delaware

No Drawing. Application September 22, 1942,  
Serial No. 459,283

14 Claims. (Cl. 204—55)

1

This invention relates to the electrodeposition of zinc, and more particularly to acid plating compositions, baths, and processes for the electrodeposition of zinc in the presence of an anthraquinone sulfonate.

Securing a good initial deposit in low current density areas upon an object being electroplated is often a difficult problem. This difficulty, commonly referred to as lack of "covering power" restricts the usefulness of many electroplating systems, since for satisfactory electroplating it is important that the object plated be covered over its entire surface with a deposit of relatively uniform thickness, and, with irregularly shaped objects, it is entirely unfeasible to distribute the current so as to avoid low current density areas. Lack of covering power is an especially troublesome problem in electroplating such metals as cast iron and malleable iron, and it has, for instance, heretofore been considered impracticable to electroplate malleable or cast iron objects with certain metals or in certain otherwise advantageous electroplating baths on account of this deficiency.

The problem of securing adequate covering power at low current densities is encountered at least to some extent in all systems for the electrodeposition of platable metals, but the need for a satisfactory answer to this problem has been particularly pressing in those systems where an important purpose of the electrodeposited metal is to protect the base metal against corrosion. Zinc is very resistant to corrosion, and accordingly with systems for the electrodeposition of zinc it is extremely important to have good covering power in all current density ranges.

Solutions for the electrodeposition of zinc may be broadly classified into two widely different categories, namely, acid-zinc baths, such as those containing zinc sulfate, and cyanide-zinc baths, such as those containing zinc cyanide, as the electrolyte in each case. By means of suitable addition agents cyanide-zinc baths have been improved in recent years so as to give bright, smooth deposits in all practical current density ranges. For some purposes such mirror-like deposits are not required and for these uses the somewhat less expensive acid-zinc baths would be suitable were it not for the fact that difficulty is encountered in securing good coverage at low current densities.

It is an object of the present invention to improve the covering power at low current densities of acid-zinc electroplating systems. A further object is to provide compositions and proc-

2

esses for the production of dense, adherent, non-porous, and ductile electrodeposits of zinc which are readily deposited in low current density areas. A further object is to provide processes for electrodepositing zinc over a variety of current densities, including low current densities, on difficultly platable objects such as irregularly shaped objects of cast or malleable iron. Further objects will become apparent hereinafter.

10 The foregoing and other objects of this invention are accomplished by processes in which zinc is electrodeposited in the presence of an anthraquinone sulfonate and are further accomplished by electrodepositing compositions and solutions in which an anthraquinone sulfonate is present.

15 The processes and compositions of this invention are characterized by their ability to effect deposition of zinc from acid baths over a wide range of densities. They are further characterized in that the deposits produced are dense, adherent, and of relatively uniform thickness. The applicability of such deposits to corrosion protection of base metals will be readily apparent.

20 Benefits are achieved according to the present invention with any acid-zinc plating baths, that is, baths having a pH lower than about 7. Acid-zinc electroplating baths may contain as the principal electrolyte, for instance, zinc sulfate or zinc chloride as shown in the examples 25 below or may contain any other salt of zinc which is stable in acid solution and is sufficiently soluble to give a substantial supply of zinc ions, such as zinc sulfamate, zinc acetate, and zinc formate.

25 The baths may be acidic by reason of the presence therein of an acid zinc salt, such as zinc sulfate, or of other acid constituents such as aluminum sulfate or chloride or ammonium chloride, or of both an acidic zinc salt and another acidic constituent. The acidity need not be great; 30 that is, the pH need not be extremely low, and may, for instance, desirably be in the range of from about 3.0 to 7.0. As already described, in such acid-zinc systems, the difficulty of getting adequate coverage at low current densities is more 35 pronounced than in alkaline baths such as cyanide-zinc baths and the benefits to be derived from the inclusion of an anthraquinone sulfonate are enhanced.

40 According to this invention any anthraquinone sulfonate may be employed in an electrodepositing composition. There may be used, for instance, monosulfonic acids, such as 1-anthraquinone sulfonic acid or 2-anthraquinone sulfonic acid, or 45 polysulfonic acids, such as 1,8-anthraquinone disulfonic acid or 2,7-anthraquinone disulfonic

acid. The bath-soluble salts of the sulfonic acids, such as sodium, potassium, or ammonium salts, or partial salts may suitably be used and because of their excellent solubility, ease of preparation, and ease of handling in dry form, the sodium salts of the sulfonic acids may be preferred. The manner of adding the sulfonic acid is comparatively unimportant, since whether the addition agent is present as an acid, or as a salt, or as a partial salt, will depend upon the pH of the bath. For purposes of this description where reference is made to a sulfonate, it will be understood that this may be a salt or partial salt or the free acid.

The amount of an anthraquinone sulfonate to include in an electroplating composition or bath will vary, depending upon the plating system involved, the metal being plated, the magnitude of effect desired, and other similar factors. The amount can best be determined by a few simple tests in the particular bath to be used. In general it will be found that from about .05 to 5.0 grams per liter of anthraquinone sulfonate will be satisfactory.

Anthraquinone sulfonates may be used in acid-zinc electroplating baths in combination with other addition agents with which they are compatible. As such additional agents, there may be used colloidal materials such as glue, wetting agents such as alcohol sulfates or naphthalene sulfonates, anti-pit agents and similar ancillary materials. When a second addition agent is used, the amount of the second agent may be considerably varied but ordinarily it should be present only in minor amount as, for instance, from about .1 to 1.0 grams per liter.

When reference is made herein to electrodeposition of zinc it will be understood that the zinc may be co-deposited with another metal or metals to produce alloys. The invention is applicable, for instance, in the co-electrodeposition of zinc and nickel or cadmium.

The invention will be better understood by reference to the following illustrative examples:

#### Example I

An acid-zinc plating bath was prepared as described in the transactions of the Electrochemical Society, vol. 80, p. 390, having the following composition:

|                                              | G./l. | Oz./gal. |
|----------------------------------------------|-------|----------|
| Zinc sulfate ( $ZnSO_4 \cdot 7H_2O$ )        | 360   | 48       |
| Ammonium chloride ( $NH_4Cl$ )               | 30    | 4        |
| Sodium acetate ( $NaC_2H_3O_2 \cdot 3H_2O$ ) | 15    | 2        |

pH adjusted to 3.5.  
Temperature 25° C.

To this bath was added 0.2 g./l. of 1-anthraquinone sodium sulfonate to obtain a bath of this invention. Copper test plates were electroplated in this bath at various current densities. It was found that complete coverage of the test plate with zinc was effected in one minute at all current densities including current densities as low as 0.1 amp./sq. ft. On the other hand similar test plates electroplated in the solution before the addition of 1-anthraquinone sodium sulfonate were not covered in one minute at current densities below about 2 to 3 amps. per square foot, indicating that the inclusion of the anthraquinone sulfonate effected an improvement in the coverage at low current densities.

#### Example II

An acid zinc plating bath was prepared as described in the transactions of the Electrochemical Society, vol. 80, p. 390, having the following composition:

|                                                  | G./l. | Oz./gal. |
|--------------------------------------------------|-------|----------|
| Zinc sulfate ( $ZnSO_4 \cdot 7H_2O$ )            | 240   | 32       |
| Ammonium chloride ( $NH_4Cl$ )                   | 15    | 2        |
| Aluminum sulfate ( $Al_2(SO_4)_3 \cdot 18H_2O$ ) | 30    | 4        |

pH adjusted to 4.0.  
Temperature 25° C.

To this bath was added 0.2 g./l. of 1-anthraquinone sodium sulfonate. Smooth white fine grained deposits were produced with excellent covering power.

#### Example III

An acid zinc plating bath was prepared as described in the transactions of the Electrochemical Society, vol. 80, p. 390, having the following composition:

|                                            | G./l. | Oz./gal. |
|--------------------------------------------|-------|----------|
| Zinc sulfate ( $ZnSO_4 \cdot 7H_2O$ )      | 410   | 43       |
| Aluminum chloride ( $AlCl_3 \cdot 6H_2O$ ) | 20    | 3        |
| Sodium sulfate ( $Na_2SO_4$ )              | 75    | 10       |

pH 3.5.  
Temperature 25° C.

To the bath was added 0.2 g./l. of 1-anthraquinone sodium sulfonate. As has been noted in previous examples, the inclusion of the anthraquinone sulfonate resulted in a decided increase in the coverage at low current densities. Smooth, dense white deposits were produced at current densities up to about 100 amp./sq. ft.

#### Example IV

An acid-zinc plating bath was prepared as described in the transactions of the Electrochemical Society, vol. 80, p. 390, having the following composition:

|                                                  | G./l. | Oz./gal. |
|--------------------------------------------------|-------|----------|
| Zinc sulfate ( $ZnSO_4 \cdot 7H_2O$ )            | 240   | 32       |
| Sodium acetate ( $NaC_2H_3O_2 \cdot 3H_2O$ )     | 15    | 2        |
| Aluminum sulfate ( $Al_2(SO_4)_3 \cdot 18H_2O$ ) | 30    | 4        |

pH 3.5.  
Temperature 25° C.

To the bath was added 0.2 g./l. of 1-anthraquinone sodium sulfonate. Smooth, dense light colored deposits were produced, with excellent covering power.

#### Example V

An acid zinc plating bath was prepared as described in the transactions of the Electrochemical Society, vol. 50, p. 211 with the following composition:

|                                            | G./l. | Oz./gal. |
|--------------------------------------------|-------|----------|
| Zinc chloride ( $ZnCl_2$ )                 | 136   | 18       |
| Ammonium chloride ( $NH_4Cl$ )             | 214   | 29       |
| Aluminum chloride ( $AlCl_3 \cdot 6H_2O$ ) | 20    | 3        |

pH adjusted to 4.0.  
Temperature 25° C.

To the bath was added 0.2 g./l. of anthraquinone sodium sulfonate to secure a bath of this invention. Copper test plates were electroplated

in this bath at various current densities. The covering power obtained in this above chloride bath was about equal to that obtained from the sulfate type bath as described in Example I. Further, the conductivity of this bath was much superior to the sulfate bath described in Example I. By use of the anthraquinone sulfonate in the above bath complete coverage was obtained at current densities as low as 0.1 amp./sq. ft. in one minute, whereas similar plates electroplated in the solution before the addition of the 1-anthraquinone sodium sulfonate were not covered under similar conditions at current densities of 2 or 3 amp./sq. ft.

*Example VI*

An acid-zinc plating bath of the chloride type was prepared as described in the transactions of the Electrochemical Society, vol. 50, p. 211, with the following composition:

|                                            | G./L. | Oz./gal. |
|--------------------------------------------|-------|----------|
| Zinc chloride ( $ZnCl_2$ )                 | 136   | 18       |
| Sodium chloride ( $NaCl$ )                 | 234   | 31       |
| Aluminum chloride ( $AlCl_3 \cdot 6H_2O$ ) | 20    | 3        |

pH 4.0.  
Temperature 25° C.

Smooth, uniform, white dense zinc deposits were produced with excellent covering power at 30 current densities up to 100 amps./sq. ft. in unagitated solutions.

By including an anthraquinone sulfonate and, optionally, another addition agent in a dry mixture of zinc salts adapted to give an acid-zinc bath upon dissolution in water, there is obtained a complete, balanced product which is ideally suited for use by the trade. Such a product may readily be dissolved to make an acid-zinc plating bath without the necessity of individually measuring or proportioning the separate constituents.

While certain illustrative compositions and processes have been shown, it will be understood that the invention is not limited thereby but that one skilled in the art, without departing from the spirit of the invention, may readily devise numerous compositions and processes for the electrodeposition of zinc in the presence of an anthraquinone sulfonate.

I claim:

1. In a process for the electrodeposition of zinc, the step comprising effecting electrodeposition of zinc from an aqueous acid-zinc electrodepositing solution in the presence of about from .05 to 5.0 grams per liter of 1-anthraquinone sodium sulfonate.

2. A zinc electrodepositing composition in dry form, comprising a zinc compound and an anthraquinone sulfonate, the proportions of anthraquinone sulfonate and other constituents being such that when the composition is dissolved in water to make a solution of suitable concentration for electroplating the anthraquinone sulfonate is present in the solution at a concentration of from .05 to 5.0 grams per liter.

3. A zinc electrodepositing composition in dry form, comprising zinc sulfate and an anthraquinone sulfonate, the proportions of anthraquinone sulfonate and other constituents being such that when the composition is dissolved in water to

make a solution of suitable concentration for electroplating the anthraquinone sulfonate is present in the solution at a concentration of from .05 to 5.0 grams per liter.

4. A zinc electrodepositing composition in dry form, comprising zinc chloride and an anthraquinone sulfonate, the proportions of anthraquinone sulfonate and other constituents being such that when the composition is dissolved in water to make a solution of suitable concentration for electroplating the anthraquinone sulfonate is present in the solution at a concentration of from .05 to 5.0 grams per liter.

5. A zinc electrodepositing composition in dry form, comprising zinc sulfamate and an anthraquinone sulfonate, the proportions of anthraquinone sulfonate and other constituents being such that when the composition is dissolved in water to make a solution of suitable concentration for electroplating the anthraquinone sulfonate is present in the solution at a concentration of from .05 to 5.0 grams per liter.

6. A zinc electrodepositing composition in dry form, comprising a zinc compound and 1-anthraquinone sodium sulfonate, the proportions of anthraquinone sulfonate and other constituents being such that when the composition is dissolved in water to make a solution of suitable concentration for electroplating the anthraquinone sulfonate is present in the solution at a concentration of from .05 to 5.0 grams per liter.

7. An aqueous zinc electrodepositing solution comprising a zinc compound and about from .05 to 5.0 grams per liter of an anthraquinone sulfonate and having a pH lower than 7.0.

8. An aqueous zinc electrodepositing solution comprising a zinc sulfate and about from .05 to 5.0 grams per liter of an anthraquinone sulfonate and having a pH lower than 7.0.

9. An aqueous zinc electrodepositing solution comprising a zinc chloride and about from .05 to 5.0 grams per liter of an anthraquinone sulfonate and having a pH lower than 7.0.

10. An aqueous zinc electrodepositing solution comprising a zinc sulfamate and about from .05 to 5.0 grams per liter of an anthraquinone sulfonate and having a pH lower than 7.0.

11. An aqueous zinc electrodepositing solution comprising a zinc compound and about from .05 to 5.0 grams per liter of 1-anthraquinone sodium sulfonate and having a pH lower than 7.0.

12. In a process for the electrodeposition of zinc, the step comprising effecting electrodeposition of zinc from an acid-zinc electrodepositing bath in the presence of about from 0.05 to 5.0 grams per liter of an anthraquinone sulfonate.

13. In a process for the electrodeposition of zinc, the step comprising effecting electrodeposition of zinc from an acid-zinc electrodepositing bath comprising zinc sulfate as the principal electrolyte, in the presence of about from 0.05 to 5.0 grams per liter of an anthraquinone sulfonate.

14. In a process for the electrodeposition of zinc, the step comprising effecting electrodeposition of zinc from an acid-zinc electrodepositing bath comprising zinc chloride as the principal electrolyte, in the presence of about from 0.05 to 5.0 grams per liter of an anthraquinone sulfonate.

ALLEN G. GRAY.